

F. M. GILMORE.  
METHOD OF APPLYING PIPE COVERING.  
APPLICATION FILED AUG. 13, 1909.

1,013,291.

Patented Jan. 2, 1912.



Witnessed:

John George Keay  
Comedolite Company

Frank M. Gilmore  
Inventor  
By his Attorney, A. H. Herkowitz

# UNITED STATES PATENT OFFICE.

FRANK MATHANUEL GILMORE, OF CHICAGO, ILLINOIS, ASSIGNOR TO H. W. JOHNS-MANVILLE COMPANY, A CORPORATION OF NEW YORK.

## METHOD OF APPLYING PIPE-COVERING.

1,013,291.

Specification of Letters Patent. Patented Jan. 2, 1912.

Application filed August 18, 1909. Serial No. 512,651.

To all whom it may concern:

Be it known that I, FRANK MATHANUEL GILMORE, a citizen of the United States of America, residing at Chicago, county of Cook, State of Illinois, have invented certain new and useful Improvements in Methods of Applying Pipe-Covering, of which the following is a specification.

My invention relates to protective coverings for pipes and is specifically designed to protect underground metallic pipes from the chemical action of the surrounding earth.

The ordinary rusting action of damp earth on metal pipe is well known, but in the alkali regions of the western States and Territories the earth has developed an acute chemical action not only on buried pipe lines recently installed there, but also on all ordinary forms of protective covering for such pipe lines, which destroys the covering and exposed pipes in a comparatively few months. Various forms of covering for such pipe lines have been tried in these regions without success heretofore, and hundreds of miles of such covering have been taken off as useless after being in place only a comparatively short time. My invention, forming a pure mineral covering hermetically sealing the pipes within it, has successfully withstood the action of the most alkaline regions.

The best form of covering at present known to me and the best method of applying it are illustrated in the accompanying sheet of drawings, in which:

Figure 1 shows a portion of a pipe line with the first element of my preferred form of coating being applied thereto. Fig. 2 is an enlarged cross section of same. Fig. 3 shows the same with the second element of the coating being spirally wound on in position. Fig. 4 is an enlarged cross section of same. Fig. 5 shows the final coating being applied, and Fig. 6 shows an enlarged cross section of a pipe line with my finished coating in place thereon.

Throughout the drawings like reference numbers indicate like parts.

1 represents a line of pipe in final position,  
2 is a coating of hot adhesive mineral com-

position such as mineral pitch or asphaltums, which I apply to the pipe preferably after the sections thereof have been jointed together and are practically in their final position. This first coating may be applied by 55 use of a brush 3, or in any other convenient manner. While the asphaltum is still warm, soft and sticky, I wind on spirally a strip or strips of asbestos paper 4, which are usually about one sixteenth of an inch thick, 60 and about six inches wide, and which have been just previously saturated with hot asphaltum. The adjacent edges of the strip overlap, preferably about half their width, so that as a result the pipe has a covering of 65 double thickness of this material. This strip is preferably wound on while the asphaltum with which it is impregnated and coated is still hot and soft so that it coalesces readily and completely with the first coating of pure asphaltum. If the impregnating asphaltum is made soft enough, the strip might be applied cold, but the best results follow when it is put on hot. After winding on this strip, I prefer to finish off the covering with another, outer coating of pure asphaltum also applied hot, by a brush 3 as before, or otherwise, preferably before the asphaltum on the asbestos paper has had time to cool or harden. The result is an integral, air tight, water tight, acid and alkali proof covering of pure mineral substances, asbestos and asphaltum, which is also tough and strong enough to withstand ordinary shocks, and the attacks of insects or other 85 living organisms as well as the chemical action of the surrounding earth and fluids.

My invention might be applied to the separate lengths of pipe before they are connected together, but the best results are obtained by making the covering absolutely continuous, as can be done only by applying it to the completed pipe line when in, or nearly in, its final position. The invention is also useful when applied to pipes in other 95 than underground positions, but reaches its highest efficiency when protected from the drying, disintegrating action of air, hot sunshine and the other influences of an exposed position, by being buried in earth or water. 100

Having, therefore, described my invention, I claim:

The method of protecting underground metallic pipes from the chemical action of the surrounding earth which comprises the following steps: first, coating the pipes with hot asphaltum; second, saturating a strip of thick asbestos paper with hot asphaltum and

applying same while the asphaltum is still soft to the pipe so as to completely envelop it; third, applying an outer coating of hot asphaltum.

FRANK MATHANUEL GILMORE.

Witnesses:

JOHN EMORY MEEK,  
JAMES CLUTE YOUNGLOVE.